

## UNITED STATES PATENT OFFICE

2,372,563

FLUXES FOR USE IN THE TREATMENT OF  
LIGHT METALS

Edward Frederick Emley, Swinton, Manchester, England, assignor to Magnesium Elektron Limited, London, England, a company of Great Britain

No Drawing. Application December 18, 1943, Serial No. 514,840. In Great Britain December 24, 1942

## 3. Claims. (Cl. 75—93)

This invention relates to fluxes used for refining and/or protecting against oxidation light metals consisting of magnesium, magnesium base alloys, and aluminium base alloys containing magnesium, all referred to hereinafter as metal. The flux of the present invention is of the inspissated type an example of which is described in the specification of British Patent No. 539,024, and which provides a pasty viscous cover or crust on the surface of the molten metal as distinct from the thinly fluid cover of the fluid type of flux. The flux of the said prior patent consists of anhydrous magnesium chloride (30—50%), chlorides of calcium, sodium, and potassium, and the inspissating agents magnesium oxide and calcium fluoride. The chloride mixture (which I term a "protective base") melts at a low temperature and protects the metal against oxidation during melting.

I have now made investigations with the object of reducing the number of ingredients in the flux with a view to cheapening its production and at the same time if possible to reducing the quantity of magnesium chloride, as this is the most expensive constituent. In these investigations I found that in the absence of magnesium oxide (or at any rate less than 5% of magnesium oxide), the calcium fluoride content requires to be between 25 and 40 per cent to ensure sufficient inspissation and to produce other desirable properties of the flux. With such percentages however it was found that low percentages of magnesium chloride gave unsatisfactory results. The proportion of calcium fluoride required to give a satisfactory consistency was found to increase rapidly with the temperature which I discovered was due to increasing solubility of the calcium fluoride in the protective base as the temperature increased. Moreover it appeared that calcium fluoride in solution in this manner in the protective base tended to prevent the flux from "wetting" the molten metal.

Attempts were made by varying the composition of the protective base to reduce its solvent power for calcium fluoride but without success.

After considerable research it was discovered that magnesium fluoride is insoluble in the protective base even at elevated temperatures and thus as calcium fluoride passes into solution magnesium fluoride is precipitated as long as magnesium chloride is present in excess. This magnesium fluoride acts as an inspissating agent and it was only necessary to have proportions of magnesium chloride in the protective base more than stoichiometrically equivalent to the calcium fluoride added to ensure that the non-wetting effect

of the calcium fluoride was avoided and also to obtain satisfactory inspissation of the protective base and a flux of good consistency at all temperatures between 650° C. and 950° C. Thus whilst magnesium chloride is usually incorporated in fluxes to increase their fluidity it may have just the opposite effect at higher temperatures when used in conjunction with calcium fluoride.

10 In this way I found it possible to produce satisfactory fluxes in which the magnesium oxide content was less than 5% whilst the magnesium chloride content is fairly low, but sufficient to be equivalent to the calcium fluoride added. In fact 15 I found that a slight excess of magnesium chloride over this equivalent was desirable. Thus, whilst 95 parts of magnesium chloride are theoretically equivalent to 78 parts calcium fluoride, I found it desirable to use 95 to 102 parts of 20 magnesium chloride to 78 parts of calcium fluoride.

Nevertheless, whilst it is preferable for the magnesium chloride to be at least stoichiometrically equivalent to the quantity of calcium fluoride, I find that in the case of fairly stiff fluxes the non-wetting tendency due to an insufficiency of magnesium chloride is masked by the viscosity and it is therefore possible to produce satisfactory fluxes containing less magnesium chloride, for example up to 40 per cent calcium fluoride with only 40 per cent magnesium chloride. Accordingly the required quantity of magnesium chloride may be regarded as at least equal in weight to the weight of fluoride.

35 I also consider that the calcium fluoride can be replaced at least partly by another fluoride or other fluorides of the alkali or alkaline earth metals.

40 Taking all the above factors into consideration I find that satisfactory fluxes can be made with in the following ranges of ingredients:

|                                                         | Per cent             |
|---------------------------------------------------------|----------------------|
| Magnesium chloride                                      | 25 to 48             |
| 45 Alkali or alkaline earth metal fluoride or fluorides | Over 25 and up to 40 |
| Magnesium oxide                                         | Less than 5          |
| Calcium chloride                                        | 5 to 27              |
| Sodium chloride                                         | Up to 20             |
| 50 Potassium chloride                                   | Up to 20             |
| Inert impurities                                        | Up to 5              |

the sodium and potassium chlorides amounting together to between six and thirty per cent, and the magnesium chloride being at least equal in weight to the weight of fluoride or fluorides.

The fluxes also do have the advantage that they do not tend to dry up so rapidly on the molten metals as fluxes containing large proportions of magnesium oxide and do not form such a hard crust if the metal is superheated. Furthermore these fluxes are more suitable than fluxes containing large proportions of magnesium oxide when used during melting where in the case for example of small melts of clean ingot, the use of more fluid fluxes is unnecessary.

Within the above quoted range the following more limited range of composition is preferred:

|                                                       | Per cent             |
|-------------------------------------------------------|----------------------|
| Alkali and alkaline earth metal fluoride or fluorides | Over 25 and up to 33 |
| Magnesium chloride                                    | 28-39                |
| Calcium chloride                                      | 9-24                 |
| Sodium chloride                                       | 5-17                 |
| Potassium chloride                                    | 3-13                 |
| Magnesium oxide                                       | Less than 5          |
| Other materials (including oxidic impurities)         | Less than 5          |

the sodium and potassium chlorides together amounting to between 12 and 24% and the magnesium chloride as before being at least equal in weight to the weight of fluoride or fluorides.

As example of specific compositions of fluxes that have been tested and found satisfactory the following are cited:

|                    |     |     |
|--------------------|-----|-----|
| Magnesium chloride | 35  | 38  |
| Calcium fluoride   | 27  | 31  |
| Magnesium oxide    | Nil | Nil |
| Calcium chloride   | 17  | 14  |
| Sodium chloride    | 13  | 11  |
| Potassium chloride | 8   | 6   |
| Inert impurities   | Nil | Nil |

The impurities may comprise barium or strontium chlorides, and oxides such as silica, iron oxide and calcium oxide.

The fluxes were examined for various characteristics including ease of stirring into the molten metal, stability of the flux cover at high tem- 40

peratures, ability to absorb the thinly fluid type flux used for initial melting of the metal, ability to absorb magnesium oxide, refining capabilities, hygroscopicity, and quantity of flux required. 5 These fluxes were found to be equally as satisfactory as those of British Patent 539,024, whilst the magnesium chloride content has been reduced. Metal was analysed for silicon both before and after treatment with flux of the present invention, and it was found that no appreciable transference of silica from the flux to the metal had occurred.

I claim:

1. A flux in which with at least one fluoride selected from the group consisting of alkali and alkaline earth metal fluorides in amount over 15 25 and up to 40%, and calcium chloride 5 to 27% of magnesium chloride 25 to 48%, there is at least one alkali metal chloride in minor amount, and the magnesium chloride being at least equal in weight to the weight of fluoride.

2. A flux having a composition within the following range:

|                                                                                                 | Per cent             |
|-------------------------------------------------------------------------------------------------|----------------------|
| At least one fluoride selected from the group consisting of alkali and alkaline earth fluorides | Over 25 and up to 33 |
| Magnesium chloride                                                                              | 28-39                |
| Calcium chloride                                                                                | 9-24                 |
| Sodium chloride                                                                                 | 5-17                 |
| Potassium chloride                                                                              | 3-13                 |
| Magnesium oxide                                                                                 | Less than 5          |
| Other materials (including oxidic impurities)                                                   | Less than 5          |

the sodium and potassium chlorides together amounting to between 12 and 24% and the magnesium chloride being at least equal in weight to the weight of fluoride.

3. A flux as claimed in claim 1 wherein calcium fluoride is the only fluoride in the composition.

EDWARD FREDERICK EMLEY.